# EUROPEAN PATENT SPECIFICATION

(11) **EP 2 604 349 B1**
(45) Date of publication and mention of the grant of the patent: **15.07.2015**
(21) Application number: 11193063.2
(22) Date of filing: 12.12.2011
(51) Int. Cl.: B05D 5/00, F41H 3/00, B05D 7/00, B05D 7/14

(54) **Method for adapting an original paint layer on an article, article having an original paint layer and a peelable, new paint layer applied thereupon.**
Methode zur Anpassung der ursprünglichen Lackschicht eines Artikels durch das Auftragen einer neuen abziehbaren Farbschicht auf dessen Oberfläche, sowie ein Artikel aufweisend die besagte abziehbare Farbschicht.
Procedé pour la modification d'un article, couvert d'une peinture originale, par le dépôt d'une couche de lacquage amovible, et un article couvert par ladite couche amovible.

(43) Date of publication of application: 19.06.2013
(73) Proprietor: Walon B.V., 4824 AG Breda (NL)
(72) Inventor: Wesselman, Joannes Franciscus Antonius, 4844 AM Terheijden (NL)
(74) Representative: van Kooij, Adriaan

(56) References cited:
- EP-A1- 0 336 196
- WO-A2-01/83878
- US-A- 5 686 145

## Description

The present invention relates to a method for adapting an original paint layer on an object, preferably on a vehicle.

For the purpose of presenting vehicles, in particular cars, on specific occasions it is often required to adapt the appearance of the vehicle to the occasion. When such a wish exists, it is then usual to adapt the appearance of a car by spraying over the original paint layer of the car with a new paint layer.

In this way it is possible to respray a car successively a number of times for different presentations. A drawback of respraying is that the new visible paint layer is applied permanently, and the original paint layer cannot be readily restored. The number of times respraying is possible is further limited because the overall paint layer increases in thickness with each treatment, while the thickness of the overall paint layer for cars is restricted.

The present invention has for its object to provide a new method which does not have the above stated drawbacks. It is also an object of the invention to achieve a similar end result in respect of the quality of the newly applied paint layer.

According to a first aspect, this object of the invention is achieved by providing a method for adapting an original paint layer on an object, preferably on a vehicle, comprising the steps of:
- arranging a resin layer on the object, subsequently allowing the resin layer to cure, wherein after curing a resin layer is obtained which is adhered peelably to the original paint layer; and
- applying a new paint layer to the peelable resin layer and allowing the paint layer to dry.

The new paint layer is similar in quality to a paint layer obtained by direct respraying as according to the prior art. The new paint layer according to the invention can moreover be peeled off the original paint layer. When a subsequent adaptation of the paint layer is required, the peelable resin layer with new paint layer can thus be first removed in its entirety from the object, after which the original paint layer is obtained. This is then provided once again with a peelable resin layer and another new paint layer without increasing the thickness of the overall paint layer. The object with original paint layer can moreover be easily restored in this way. This method of operation provides an attractive and advantageous way of varying the paint colours of the object.

Curing of the resin layer can be achieved by drying in air, optionally at increased temperature.

It is noted by the way that peelable resin layers are per se known in the field, particularly as protective layers on vehicles (see for example EP 0 336 196 A1 and WO 01/83878 A2) . Other functionalities of the peelable resin layers are also known, wherein the peelable resin layer itself has for instance a camouflage colour or camouflage pattern for the purpose of military vehicles.

Applying a separate new paint layer to a peelable resin layer has however not been described, nor has it been previously suggested.

The method according to the invention preferably comprises a subsequent additional step of:
- applying a transparent top layer to the new paint layer and allowing the top layer to dry.

An optimum end result is thus obtained wherein the new paint layer has the appearance of an original paint layer, wherein the top layer moreover fulfils a protective function.

In the method according to the invention one or more of the applied layers are more preferably applied by spraying on a liquid.

Spraying on a liquid is a very practical method of applying the respective layers. Each layer can thus be applied as a thin film.

With particular preference the method according to the invention comprises a prior additional step of:
- pretreating the upper surface of the original paint layer by cleaning and drying thereof.

This makes it possible to arrange an optimal, even film of peelable resin layer, so that the subsequently applied new paint layer has the appearance of an original paint layer.

It is further recommended in the method according to the invention that the peelable resin layer is of a type classified as tacky booth coating.

In the relevant field tacky booth coatings are known and extensively described as a coating suitable for covering inner walls of spray booths. This type of coating is commercially available in different variants. The coating is sprayed as a protective layer on the inner walls of the spray booths and cured. The material has a decreased adhesive power and can therefore be peeled off the inner wall. The protective layer serves to collect residues of sprayed paints which have not settled on the object for spraying in the spray booth. The protective layer can be peeled off at any desired moment and replaced by a new protective layer. The inner walls of a spray booth are thus permanently protected from residues of paints which have not settled on the object for spraying.

It has been found that a peelable resin layer of the tacky booth coating type is highly suitable for the method according to the invention.

In addition, it is recommended in the method according to the invention that the peelable resin layer comprises as main component a partially cured resin chosen from the group of polyurethane, polyvinyl butyral, ethylene vinyl acetate, ethylene acrylate, polyvinyl acetate and the derivatives thereof, as well as combinations of the above stated resins and their derivatives.

Such a resin is found to function very well as underlayer for the new paint layer, while at the same time having good peelability relative to the original paint layer. A shared feature of these resins is that they do not cure completely, whereby a fraction of unreacted groups is present in the resin layer. This fraction of unreacted groups is also present in the contact surface of the resin layer lying against the original paint layer. The resin layer can be peeled off on this basis.

In the method according to the invention the resin layer is more preferably arranged in the form of an aqueous suspension of the reactants for the corresponding resin.

An aqueous suspension is recommended because it generally has little environmental impact, and the health hazards are moreover reduced for those applying the resin layer. The aqueous suspension is moreover suitable for spraying on of a resin layer.

The reactants for the resin depend of course on the type of resin chosen: for polyurethane these are isocyanate and glycol; for polyvinyl butyral they are polyvinyl alcohol and butanal; for polyvinyl acetate this is the monomer vinyl acetate; for ethylene vinyl acetate and ethylene acrylate they are the corresponding monomers, i.e. ethylene and vinyl acetate, and vinyl acrylate respectively.

The reactants for the resin can alternatively be a prepolymer of the resin. It is also possible for the reactants of the resin to be a mixture of the corresponding monomers and the corresponding prepolymer.

It is also recommended in the method according to the invention that the resin layer, in the form in which it is arranged, comprises additives of surfactants and/or release agents.

Such additives increase the suitability of the reactants for the resin to be arranged in the form of a liquid.

In the method according to the invention a cured resin layer is with particular preference obtained which comprises as additive a pigment, preferably a white pigment.

Such a resin layer forms a suitable surface for applying a new paint layer because the white pigment prevents the colour of the underlying original paint layer showing through, thereby avoiding a show-through effect on the new paint layer.

It is recommended in the method according to the invention that the cured resin layer has a thickness in the range of 10 to 50 micrometres, and preferably 15 to 40 micrometres. This thickness has been found highly suitable for meeting all the requirements of a peelable layer in the context of the invention.

It is noted for the sake of completeness that the new paint layer applied to the peelable resin layer preferably has a thickness in the range of 15-25 micrometres, and the optional top layer has a thickness in the range of 40-50 micrometres.

According to a second aspect of the invention, an object is provided, preferably a vehicle, which is provided with an original paint layer on which the following successive layers are present:
- a cured, peelable resin layer, and
- a dried, new paint layer.

Such an object is highly suitable for use in presentations wherein the object is provided with a temporary paint layer desired for the presentation. The object can be shown again with the original paint layer by peeling off the peelable resin layer to which the temporary paint layer has been applied. If desired, warm water can be applied during peeling in order to simplify peeling or to remove residues of the resin layer left behind.

Several recommended variants of the object according to the invention follow below. The advantages of these variants have already been elucidated above with reference to the method according to the invention.

In the case of the object according to the invention a dried transparent top layer is preferably present on the new paint layer.

In the case of the object according to the invention the peelable resin layer is more preferably of a type classified as tacky booth coating.

According to a following variant, the peelable resin layer comprises as main component a partially cured resin chosen from the group of polyurethane, polyvinyl butyral, ethylene vinyl acetate, ethylene acrylate, polyvinyl acetate and the derivatives thereof, as well as combinations of the above stated resins and their derivatives.

The cured resin layer preferably further comprises as additive a pigment, more preferably a white pigment.

The cured resin layer preferably has a thickness in the range of 10 to 50 micrometres, and preferably 15 to 40 micrometres.

## Claims

1. Method for adapting an original paint layer on an object comprising the steps of:
- arranging a resin layer on the object, subsequently allowing the resin layer to cure, wherein after curing a resin layer is obtained which is adhered peelably to the original paint layer; and
- applying a new paint layer to the peelable resin layer and allowing the paint layer to dry,
wherein the resin comprises a partially cured resin chosen from the group of polyvinyl butyral, ethylene vinyl acetate, ethylene acrylate, polyvinyl acetate and derivatives thereof, as well as combinations of the above stated resins and their derivatives.

2. Method as claimed in claim 1, with a subsequent additional step of:
- applying a transparent top layer to the new paint layer and allowing the top layer to dry.

3. Method as claimed in any of the foregoing claims, wherein one or more of the applied layers are applied by spraying on a liquid.

4. Method as claimed in any of the foregoing claims, with a prior additional step of:
- pretreating the upper surface of the original paint layer by cleaning and drying thereof.

5. Method as claimed in any of the foregoing claims, wherein the paint layer is applied with thickness of 15-25 micrometers.

6. Method as claimed in any of the foregoing claims, wherein the object is a vehicle.

7. Method as claimed in any of the foregoing claims, wherein the resin layer is arranged in the form of an aqueous suspension of the reactants for the corresponding resin.

8. Method as claimed in any of the foregoing claims, wherein the resin layer, in the form in which it is arranged, comprises additives of surfactants and/or release agents.

9. Method as claimed in any of the foregoing claims, wherein a cured resin layer is obtained which comprises as additive a pigment, preferably a white pigment.

10. Method as claimed in any of the foregoing claims, wherein the cured resin layer has a thickness in the range of 10 to 50 micrometres, and preferably 15 to 40 micrometres.

11. Objectprovided with an original paint layer on which the following successive layers are present:
- a cured, peelable resin layer, wherein the resin comprises a partially cured resin chosen from the group polyvinyl butyral, ethylene vinyl acetate, ethylene acrylate, polyvinyl acetate and derivatives thereof, as well as combinations of the above stated resins and their derivatives, and
- a dried, new paint layer.

12. Object as claimed in claim 11, wherein a dried transparent top layer is present on the new paint layer.

13. Object as claimed in claim 11 or 12, wherein the peelable resin layer is a coating suitable for covering inner walls of spray booths.

14. Object as claimed in any of the foregoing claims 11-13, wherein the cured resin layer comprises as additive a pigment, preferably a white pigment.

15. Object as claimed in any of the foregoing claims 11-14, wherein the cured resin layer has a thickness in the range of 10 to 50 micrometres, and preferably 15 to 40 micrometres.

16. Object as claimed in claim 11, wherein the object is a vehicle.

## Patentansprüche

1. Verfahren zum Anpassen einer ursprünglichen Anstrichmittelschicht auf einem Gegenstand, welches die Schritte umfasst:
- Anordnen einer Harzschicht auf dem Gegenstand, nachfolgend Härtenlassen der Harzschicht, wobei nach dem Härten eine Harzschicht erhalten wird, die an der ursprünglichen Anstrichmittelschicht abziehbar angeheftet ist, und
- Auftragen einer neuen Anstrichmittelschicht auf die abziehbare Harzschicht und Trocknenlassen der Anstrichmittelschicht,
wobei das Harz ein teilweise gehärtetes Harz, ausgewählt aus der Gruppe von Polyvinylbutyral, Ethylenvinylacetat, Ethylenacrylat, Polyvinylacetat und Derivaten davon sowie auch Kombinationen der oben angegebenen Harze und von deren Derivaten, umfasst.

2. Verfahren nach Anspruch 1 mit einem nachfolgenden zusätzlichen Schritt eines:
- Auftragens einer transparenten Deckschicht auf die neue Anstrichmittelschicht und Trocknenlassen der Deckschicht.

3. Verfahren nach einem der vorangegangenen Ansprüche, wobei eine oder mehrere der aufgetragenen Schichten durch Aufsprühen einer Flüssigkeit aufgetragen werden.

4. Verfahren nach einem der vorangegangenen Ansprüche mit einem vorher durchzuführenden zusätzlichen Schritt eines:
- Vorbehandelns der oberen Oberfläche der ursprünglichen Anstrichmittelschicht durch Reinigen und Trocknen von dieser.

5. Verfahren nach einem der vorangegangenen Ansprüche, wobei die Anstrichmittelschicht mit einer Dicke von 15-25 Mikrometern aufgetragen wird.

6. Verfahren nach einem der vorangegangenen Ansprüche, wobei der Gegenstand ein Fahrzeug ist.

7. Verfahren nach einem der vorangegangenen Ansprüche, wobei die Harzschicht in Form einer wässrigen Suspension der Reaktanten für das entsprechende Harz angeordnet wird.

8. Verfahren nach einem der vorangegangenen Ansprüche, wobei die Harzschicht in der Form, in der sie angeordnet wird, Zusätze von grenzflächenaktiven Mitteln und/oder Trennmitteln umfasst.

9. Verfahren nach einem der vorangegangenen Ansprüche, wobei eine gehärtete Harzschicht erhalten wird, die als Zusatz ein Pigment, vorzugsweise ein weißes Pigment, umfasst.

10. Verfahren nach einem der vorangegangenen Ansprüche, wobei die gehärtete Harzschicht eine Dicke im Bereich von 10 bis 50 Mikrometern und vorzugsweise 15 bis 40 Mikrometern aufweist.

11. Gegenstand, der versehen ist mit einer ursprünglichen Anstrichmittelschicht, auf welcher die folgenden aufeinanderfolgenden Schichten vorhanden sind:
- eine gehärtete, abziehbare Harzschicht,
wobei das Harz ein teilweise gehärtetes Harz, ausgewählt aus der Gruppe von Polyvinylbutyral, Ethylenvinylacetat, Ethylenacrylat, Polyvinylacetat und Derivaten davon sowie auch Kombinationen der oben angegebenen Harze und von deren Derivaten, umfasst, und
- eine getrocknete neue Anstrichmittelschicht.

12. Gegenstand nach Anspruch 11, wobei eine getrocknete transparente Deckschicht auf der neuen Anstrichmittelschicht vorhanden ist.

13. Gegenstand nach Anspruch 11 oder 12, wobei die abziehbare Harzschicht eine Beschichtung ist, die zum Überziehen von inneren Wänden von Spritzkabinen geeignet ist.

14. Gegenstand nach einem der vorangegangenen Ansprüche 11-13, wobei die gehärtete Harzschicht als Zusatz ein Pigment, vorzugsweise ein weißes Pigment umfasst.

15. Gegenstand nach einem der vorangegangenen Ansprüche 11-14, wobei die gehärtete Harzschicht eine Dicke im Bereich von 10 bis 50 Mikrometern und vorzugsweise 15 bis 40 Mikrometern aufweist.

16. Gegenstand nach Anspruch 11, wobei der Gegenstand ein Fahrzeug ist.

## Revendications

1. Procédé destiné à adapter une couche de peinture d'origine sur un objet, comprenant les étapes consistant à :
- agencer une couche de résine sur l'objet, et permettre ensuite à la couche de résine de durcir, dans lequel, après le durcissement, on obtient une couche de résine qui adhère de manière pelable à la couche de peinture d'origine ; et
- appliquer une nouvelle couche de peinture sur la couche de résine pelable et laisser la couche de peinture sécher ;
dans lequel la résine comprend une résine durcie en partie sélectionnée dans le groupe constitué par : un butyral de polyvinyle, un éthylène - acétate de vinyle, un acrylate d'éthylène, un acétate de polyvinyle et des dérivés de ceux-ci, ainsi que des combinaisons de résines mentionnées ci-dessus et des dérivés de celles-ci.

2. Procédé selon la revendication 1, comprenant une étape supplémentaire suivante consistant à :
- appliquer une couche supérieure transparente sur la nouvelle couche de peinture et permettre à la couche supérieure de sécher.

3. Procédé selon l'une quelconque des revendications précédentes, dans lequel une ou plusieurs des couches appliquées sont appliquées par pulvérisation d'un liquide.

4. Procédé selon l'une quelconque des revendications précédentes, comprenant une étape supplémentaire précédente consistant à :
- traiter au préalable la surface supérieure de la couche de peinture d'origine en la nettoyant et en la séchant.

5. Procédé selon l'une quelconque des revendications précédentes, dans lequel la couche de peinture est appliquée avec une épaisseur comprise entre 15 micromètres et 25 micromètres.

6. Procédé selon l'une quelconque des revendications précédentes, dans lequel l'objet est un véhicule.

7. Procédé selon l'une quelconque des revendications précédentes, dans lequel la couche de résine est agencée sous la forme d'une suspension aqueuse de réactifs de la résine correspondante.

8. Procédé selon l'une quelconque des revendications précédentes, dans lequel la couche de résine, dans la forme selon laquelle elle est agencée, comprend des additifs d'agents tensio-actifs et / ou d'agents antiadhésifs.

9. Procédé selon l'une quelconque des revendications précédentes, dans lequel on obtient une couche de résine durcie qui comprend, en tant qu'additif, un pigment, de préférence un pigment blanc.

10. Procédé selon l'une quelconque des revendications précédentes, dans lequel la couche de résine durcie présente une épaisseur qui se situe dans une plage comprise entre 10 micromètres et 50 micromètres, et comprise de préférence entre 15 micromètres et 40 micromètres.

11. Objet doté d'une couche de peinture d'origine sur laquelle les couches successives suivantes sont présentes :
- une couche de résine pelable et durcie ;
dans lequel la résine comprend une résine durcie en partie sélectionnée dans le groupe constitué par : un butyral de polyvinyle, un éthylène - acétate de vinyle, un acrylate d'éthylène, un acétate de polyvinyle et des dérivés de ceux-ci, ainsi que des combinaisons de résines mentionnées ci-dessus et des dérivés de celles-ci ; et
- une nouvelle couche de peinture, séchée.

12. Objet selon la revendication 11, dans lequel une couche supérieure transparente séchée est présente sur la couche d'une nouvelle peinture.

13. Objet selon la revendication 11 ou la revendication 12, dans lequel la couche de résine pelable est un revêtement approprié au recouvrement des parois intérieures de cabines de pulvérisation.

14. Objet selon l'une quelconque des revendications 11 à 13, dans lequel la couche de résine durcie comprend, en tant qu'additif, un pigment, de préférence un pigment blanc.

15. Objet selon l'une quelconque des revendications 11 à 14, dans lequel la couche de résine durcie présente une épaisseur qui se situe dans une plage comprise entre 10 micromètres et 50 micromètres, et comprise de préférence entre 15 micromètres et 40 micromètres.

16. Objet selon la revendication 11, dans lequel l'objet est un véhicule.
